

Dec. 7, 1943.

W. J. KRUPPA

2,336,151

PRESSURE TREATMENT OF COKING COALS

Filed July 2, 1940



## UNITED STATES PATENT OFFICE

2,336,151

## PRESSURE TREATMENT OF COKING COALS

William Joseph Kruppa, Hamden, Conn., assignor,  
by mesne assignments, to American Cyanamid  
Company, New York, N. Y., a corporation of  
Maine

Application July 2, 1940, Serial No. 343,518

10 Claims. (Cl. 202—20)

The present invention relates to the treatment of coking coals and more particularly it relates to an improved method for the oxidation of badly swelling and caking coals to alter the coking characteristics thereof.

Many bituminous coals such as high volatile bituminous coals, cake and swell badly when it is attempted to carbonize them. It has been proposed in the past to reduce the caking and swelling characteristics of such coals by oxidation. In these oxidation processes it is necessary that the oxidation be controlled so that the coal when carbonized will have sufficient caking characteristics to form a firm bond during carbonization. The prior proposed methods of oxidizing such coals have the serious disadvantage that the temperature of the coal must be raised to about 150° C. and maintained at that temperature for a period of 24 to 120 hours depending upon the type of coal being treated. The prior oxidation processes are difficult to control accurately.

In accordance with the present invention I have found that even the most strongly caking and swelling coals can be oxidized to the desired reduction of its caking powers in a very much shorter time and under conditions which are more easily controlled than the proposed prior oxidation processes. My improved method broadly comprises subjecting ground coal to an oxidation treatment at elevated temperatures and pressures. Satisfactory oxidation is accomplished with many coals in from 3 to 6 hours by employing a temperature of about 150° C. and carrying the oxidation out in a tightly sealed vessel under air pressure of about 50 lbs. per square inch. In general as the pressure is decreased for a given coal the amount of swelling inhibition in a unit of time is likewise decreased. The pressure and time of treatment varies with the coal being treated. Most bituminous coals can be treated sufficiently, to produce non-swollen carbonized briquettes with coal tar or pitch as a binder, in a period of 4 hours at 50 lbs. air pressure per square inch at a temperature of 150° C. Some coals, however, do not require more than 20 lbs. air pressure per square inch and 4 hours treatment at 150° C. Other coals do not require temperatures as high as 150° C., while some coals require temperatures somewhat higher. In the coals tested the highest temperature required was about 200° C. and the lowest was about 115° C.

In general, it appears that the treatment of coal under air pressure speeds up the rate of oxidation. I have found, however, that pressures of

over 50 lbs. per square inch have very little effect on increasing the rate of oxidation, i. e., the rate of oxidation increases with the pressure up to its maximum of about 50 lbs. per square inch after which further increase in pressure does not produce a further substantial reduction in the time requirement. Pressures higher than 50 lbs. per square inch are required only with coals that require larger quantities of oxygen to bring about the desired swelling inhibition, than can be forced into the pressure treating vessel at 50 lbs. per square inch. One type of coal, for example, could not be sufficiently oxidized in 4 hours with 45 lbs. per square inch pressure unless the air in the treating vessel was changed several times. However, when this coal was treated for 4 hours at 150 lbs. pressure no air change was required indicating that the increased pressure in this case served only to supply sufficient oxygen to produce the same effect in the same time which 45 lbs. pressure produced when the air in the coal container was changed several times. Apparently the effect of this air change was to supply the coal with sufficient oxygen to bring about the desired reduction of the coal's swelling characteristics.

If the air is mixed with oxygen or if oxygen gas is used alone the temperature and pressure may be adjusted to bring about the desired changes in which case the time may be decreased or the temperature and pressure decreased. In place of air, oxygen, oxygen mixtures or other suitable oxidizing gases may be used or mixtures of such gases, air being preferred because of its cheapness.

The present invention is not limited to any particular fineness to which the coal is ground. I have found however that it has an effect on the time of treatment required under the same conditions of pressure and temperature. The temperature also has an effect on the time of treatment, in general the higher the temperature the shorter the time of treatment required. Reasonable changes in the fineness of the coal and the temperature are not as effective in reducing the time requirement for sufficient oxidation as increasing the pressure from atmospheric to 50 lbs. per square inch. This is one of the important advantages of the present invention as it permits the degree of oxidation to be very easily and accurately controlled in applying the process to different oxidation requirements.

The process is interfered with somewhat by coals that give off moisture or volatiles during the

treating process. When such coals are to be treated they are first thoroughly dried and raised to the oxidizing temperature before the pressure treatment begins. The oxidation process is more easily controlled and results are more consistent. Many coals, however, which are dry or contain very little volatile substance can be treated directly without first drying. Without limiting the invention by a particular explanation the interference is probably due to the fact that some coals more than others start to decompose about 100° C. and give off water along with other volatile constituents as the temperature is raised. This water is not surface moisture alone but the result of the decomposition of some part of the coal itself. With some coals it has been found that when put into a tightly sealed coal pressure treater and the temperature raised to about 150° C. with no provision for the escape of moisture consistent results are not obtained with the pressure treatment oxidation process. However, when these coals were first dried and raised to the desired temperature in an air stream outside the coal treater and then put into the coal treater and given a pressure treatment, satisfactory and consistent results were always attainable. In a preferred embodiment of the present invention, therefore, it is important that the coal be dried and brought up to the reacting temperature to eliminate the moisture, both external and internal before the pressure treatment begins. Briefly my improved process is carried out as follows: The coal is dried, ground to proper fineness and brought up to the desired reacting temperature (115-200° C. depending upon the coal and the final state of oxidation required) outside the pressure treater. In this step all of the surface moisture and that of constitution formed by decomposing of some part of the coal are removed from the coal mass. The hot dry coal is charged into an insulated container which is then tightly sealed and subjected to air or oxidizing gases at an elevated pressure of from 20 to 150 lbs. per square inch depending upon the coal being treated and the final state of oxidation required. The coal is allowed to remain under this pressure and at substantially the same temperature (115-200° C.) at which it was introduced into the container for a period of about 4 hours or less depending upon the coal and the final state of oxidation and swelling inhibition desired. After the required lapse of time the coal is discharged from the pressure treating container and is ready for any suitable carbonization treatment.

The invention will be described more particularly in conjunction with the drawing which is a semi-diagrammatic elevation of suitable plant for carrying out the process. It should be understood, however, that in its broader aspects the present invention is not concerned with any particular plant for carrying out the process, and the drawing represents only one such suitable plant arrangement.

In describing the method of carrying out the present invention in connection with the drawing the description relates specifically to the treatment of a badly swelling and caking Pittsburgh seam coal, containing about 35% volatile matter, and which is to be oxidized to such an extent that the treated coal can be made into coal tar pitch briquettes and carbonized at a rate of about 2 1/2° C. per minute through the plastic temperature range without swelling. The coal as delivered to the plant is of low surface moisture content.

The coal is fed into the pulverizer 1 by means of a suitable feeder 2 as illustrated in the drawing. The coal in the pulverizer is ground so that the material finer than 20 mesh is picked up by the stream of air entering the pulverizer from the larger fan 3. The temperature in the mill is controlled by an admixture of more or less of hot flue gases produced in the adjoining pulverizer furnace 4 by a combustion of coal, oil or gas. The air sweeps through the upper portion 5 of the pulverizer which contains suitable separation equipment as an integral part of the mill, the oversize dropping out of the air stream and returning to the grinding elements of the pulverizer. The air stream leaving the mill is conducted by means of the conduits 6 to a cyclone type dust collector 7 where about 90 to 95% of the coal is separated from the hot air, the remainder returning to the larger fan and thus to the mill for recirculation.

A smaller fan 8 removes air from the system and blows it through the concentrator collectors 9 where the remaining coal is substantially all removed and the waste air is then passed to the atmosphere. The fine coal collected in these concentrators is returned to the mill as shown. The amount of air passing through the concentrator collectors 9 is the same as the amount drawn into the system from the pulverizer furnace 4 plus the water evaporated from the coal, plus the water formed by decomposition of some of the coal.

The coal in the cyclone collector 7 is dry and at a temperature equal to or somewhat lower than that desired in the treaters. The temperature is controlled by the amount and temperature of flue gas drawn into the pulverizer 1 from the pulverizer furnace 4. A screen analysis of this coal shows it to range in particle size from about 88% less than 28 mesh to about 10% less than 200 mesh.

This hot coal is then fed out of the bottom of the cyclone collector 7 by means of a pulverized coal pump 10. In order to pump the pulverized coal and cause it to travel through a conveyor pipe 11 the coal is aerated by the introduction of air through the air line 12 into the coal conduit as shown. The amount of air required for proper aeration is on the order of about 5% by weight of the coal conveyed. This air required for aeration is first heated to any desired temperature in the air heater coil 13 and provides one method of producing accurate temperature control of the coal before its introduction into the coal treaters.

The coal is conveyed through the conduit 11 to the coal treaters 14. This conduit is preferably jacketed and steam or oil at temperatures of 150° C. or more is introduced into the jacket to further raise or control the coal temperature desired. The length of this conduit and the temperature of steam or oil used in its jacket is sufficient to assure the delivery of coal at exactly the proper temperature, in this example 150° C., to the coal treaters 14.

The treaters 14 are simple insulated tanks capable of withstanding 50 lbs. per square inch pressure. In a large plant there would be a number of treaters as shown and in a smaller plant perhaps only two or even one. When the first treater is filled, the coal valve 15 in the coal conduit is closed and the valve to the next treater is opened. The first treater is immediately put under 50 lbs. per square inch air pressure and allowed to stand for 4 hours under that pressure.

The air introduced into the treaters may or may not be preheated. It is an advantage however that hot air can be used as the temperature of the coal is more easily maintained. The air may also be mixed with oxidizing gases if desired.

After an elapsed time of about 4 hours the coal is discharged from the coal treater 14 into the treated coal bin 16 from whence a suitable feeder 17 conveys the treated coal to the fluxing and briquetting equipment. The badly swelling and caking bituminous coals which normally cannot be successfully coked are in accordance with the present invention altered to such an extent that they can be coked by any of the ordinary carbonization processes. Because of the desirability, however, for finely grinding the coal in carrying out my processes the practical methods of coking should be limited to compressing, briquetting, and agglomerating processes prior to carbonization. In the case of briquettes the coal can be compressed into a briquette with or without a binder and carbonized at an intense rate to obtain a compact and unswollen briquette. In agglomerating processes the coal after oxidation can be fluxed with a small amount of cheap adhesive and rolled through a tubular mill to agglomerate it into balls which can then be charged into an ordinary coking oven and coked without interference of swelling or caking while passing through the plastic temperature range.

In the manufacture of briquettes from the bituminous coals there are at least two difficulties which are encountered: first, the coal has a tendency to be plastic and swells and this results in the production of a very poorly formed briquette of low specific gravity and in many instances the caking tendency is so strong that the briquettes cannot be separated one from another; secondly, the compressed briquettes must have sufficient head load bearing strength so that the underlying briquettes will not be crushed by the weight of the briquettes above them.

The preoxidation treatment of the present invention overcomes the difficulties due to caking and swelling. The head load bearing ability of the briquettes is not extensively associated with oxidation. It is an advantage of the present invention however that the pre-oxidation does not reduce the head load bearing ability of briquettes and in some instances increases it so that the binders usually employed in manufacturing briquettes from a good quality coking coal can be used with my pre-oxidized coal and moreover the degree of oxidation can be controlled so that the coking characteristics of the coal may be more readily amenable to the use of various binders; for example, a highly swelling coking coal can be oxidized to the point that the coking characteristics of the coal are changed to something on the order of a Beckley seam coal and sulfite liquor can be used as a binder. In this type of coal there is still enough plasticity remaining so that the briquettes are firmly bound by the sulfite liquor and they will bear a sufficient head load. Such coal, however, cannot be successfully used with pitch and tar binders to produce a briquette having suitable head load bearing ability. If pitch or tar is to be used as a binder the coal is preferably oxidized to such an extent that it corresponds to "Peace and partner's" "A" and "B" coals. These are British weakly coking coals, the "A" described as "Thorne dry cleaned smalls" containing about 36.1% volatiles, 58.5% fixed carbon and 5.4% ash. "B" is described as "Alerton main washed smalls" containing about 35.6% vol-

5 atiles, 58.8% fixed carbon and 5.6% ash. Irrespective of the head load bearing ability of the briquettes and the binders used the pre-oxidation changes the coking characteristics of the badly swelling caking coals so that they can be carbonized at the rate of at least  $2\frac{1}{2}$ ° C. per minute through the plastic range as contrasted to untreated coals in which the temperature rise cannot be more than about  $\frac{1}{2}$ ° C. per minute through the plastic temperature range.

10 It is therefore an advantage of the present invention that when badly caking or coking coal is oxidized the coking characteristics of the coal are altered to such an extent that when briquetted the briquettes can be carbonized at higher rates of temperature rise through the plastic temperature range without fusing, swelling, sticking together or slumping. It has been found that the extent of oxidation required to achieve this end varies somewhat with the binder to be used in the briquetting operation. When coal tar or pitch is used as a binder the oxidation should be carried to such an extent that a test briquette of the oxidized coal containing no binder will carbonize at a temperature rise rate of  $2\frac{1}{2}$ ° C. per minute through the plastic temperature range to produce an unswollen and only slightly bonded carbonized product. When sulfite liquor is used as a binder the oxidation does not necessarily have to be carried out to quite such an extent, and some swelling in the non-binder briquette test is allowed. When molasses or other carbohydrate material is used as a binder the degree of oxidation should be approximately the same as for sulfite liquor. In general it has been found that with all other conditions being the same the time of oxidation treatment to produce sufficient swelling inhibition when sulfite liquor binder is used is only about  $\frac{3}{4}$  of that required to produce sufficient inhibition with coal tar or pitch as a binder.

15 The following specific tests carried out on different coking coals will serve to further illustrate the operativeness of the present invention and also the flexibility of the invention when applied to different coking coals.

20 The following tests were conducted on the "Hillman Coal Company's emerald coal" and "Berwind-White's ocean coal," both of which are Pittsburgh seam coals and are highly swelling, highly melting coals. These coals cannot be run in ordinary briquetting carbonization plants at a temperature rise of more than  $\frac{1}{2}$ ° C. per minute through the plastic temperature range and will not bear more than a 4 foot head load using sulfite liquor.

25 The coals were first ground so that about 90% passed through a 28 mesh screen, the ground coal was then dried at a temperature of about 150° C. until all of the surface moisture and that of constitution formed at or below 150° C. had been removed. The hot dry coal was then charged into the pressure treaters and subjected to a pressure of 50 lbs. per square inch at the temperature of 150° C. for a period of 4 hours.

30 Briquettes were made from the treated coal using no binders and while the binding properties were not very good the briquettes could be carbonized at a temperature rise of from  $2\frac{1}{2}$  to 6° C. rise per minute through the plastic temperature range without any undue swelling and caking, to produce briquettes of good density.

35 Briquettes were also made from the treated coal using 4% sulfite liquor dry substance as a binder and subjected to carbonization. The sulfite liquor bound briquettes were unswollen, well

bonded, had sufficient head load strength to bear a six foot head load and produced briquettes of good density. Briquettes were likewise made from the treated coal using 4% molasses as a binding substance. The briquettes were well bonded and upon carbonization the swelling and caking was satisfactory in that the carbonization could be carried out at a temperature rise of at least  $2\frac{1}{2}$ ° C. per minute through the plastic temperature range but the head load bearing strength was somewhat weaker. The pretreated coal when made into briquettes using about 5% pitch or coal tar as a binding material produced briquettes having a good bond and excellent swelling and coking properties but with poor head load resistance. Upon experimentation it was discovered that if the pitch or coal tar bound briquettes were heated in air at a temperature of about 200 to 240° C. for a period of from 15 minutes to 1 hour prior to the carbonization treatment the briquettes had excellent head load bearing strength.

This heat treatment in an oxidizing atmosphere of the tar or pitch bound briquettes previous to their carbonization is an important step in briquetting operations using the pre-oxidized coals of the present invention. Tar and pitch are by-products of caking operations and are therefore not only readily available but are also cheap. Tar and pitch bound briquettes however are not suitable in general for carbonization processes in which the briquettes must bear a super-imposed head load, i. e., they have very poor head load strength, but if these briquettes are first heated in an oxidizing atmosphere for from 15 minutes to 1 hour at a temperature from 200 to 240° C. they will bear super-imposed loads up to 6 feet and thus make their carbonization in large quantities a practical process.

The above tests were also carried out on a straight Beckley coal which is considered to be a coking coal well adapted for forming briquettes. In each instance the pre-treated Pittsburgh seam coals resulted in the production of briquettes which were equivalent in quality to those produced from the Beckley coal and in most instances were of a better quality.

Tests were also conducted on certain British coals of the "Peace and partner's" class. Some of these coals, specifically "A" and "B" can be successfully run at economical rates in briquetting processes without pretreatment, however, the coals "C," "E," and "F" cannot be made into briquettes and carbonized by the usual processes because of their extreme swelling characteristics. Coal "C" is described as "Thirlsington washed nuts" containing about 33.2% volatiles, 63.8% fixed carbon, 3.00% ash and is strongly coking.

"E" is described as "Waterhouse's unwashed coal" containing about 26.4% volatiles, 69.6% fixed carbon, 4.00% ash and is strongly coking. "F" is strongly coking low ash coal containing about 28.3% volatiles, 68.9% fixed carbon and 2.80% ash. When the "C," "E," and "F" coals are pre-treated in accordance with the present invention the swelling properties are altered to such an extent that they can economically be briquetted and carbonized. The treatment of these 3 coals followed the same general procedure as that described in connection with the Pittsburgh seam coals with only slight variations to compensate for the degree of oxidation to which each of the coals should be subjected. For example, coal "C" was ground and dried

at a temperature of about 115° C. and charged into the pressure treater and held at a temperature of 115° C. for 3 hours under 50 lbs. per square inch air pressure. The briquettes from this coal bound with 4% sulfite liquor dry substance and carbonized at  $2\frac{1}{2}$ ° C. rise per minute through the plastic temperature range produced very hard, clean, undistorted briquettes with a diametric shrinkage of about 7%. Coal "E" was subjected to the same treatment as coal "C" and produced equally excellent sulfite liquor bound briquettes being very hard, dense, clean, undistorted and with a diametric shrinkage of about 5%. Coal "F" when subjected to oxidation under conditions similar to coals "C" and "E" could not be economically carbonized in the form of briquettes and the oxidation procedure was accordingly altered somewhat. The coal "F" was ground and dried at a temperature of 150° C. for 4 hours under 45 lbs. air pressure while at the same time allowing a small quantity of air to bleed through the coal and then out of the container. Briquettes made from this treated coal with 4% sulfite liquor dry substance and carbonized at  $2\frac{1}{2}$ ° C. rise per minute through the plastic temperature range were very hard, dense, and clean with a diametric shrinkage of about 8%. Briquettes made without binders were unswollen and poorly bonded which shows that the treatment destroyed almost completely the fusing property of the coal. The above treatment of coal "F" indicates that there was insufficient oxygen present at a pressure of 50 lbs. and at a temperature of 150° C. to sufficiently alter the caking characteristics of the coal and hence the bleeding of air through the coal during the pressure treatment served to supply the necessary oxygen. This is further evidenced by the fact that the same coal ground and dried at a temperature of 150° C. and then subjected to air pressure of 150 lbs. per square inch and held at the temperature of 150° C. for 4 hours resulted in the production of oxidized coal which could be successfully briquetted. This type of coal can be altered more readily by using a gas having stronger oxidizing properties than air.

Tests were conducted on the pre-treated coals "C," "E," and "F" in briquetting operation using binders other than sulfite liquor. The results in general are the same as previously described in connection with the Pittsburgh seam coals.

The present invention is of course not limited to the treatment of the particular coals as described but is generally adaptable for the treatment of coals capable of coking but which because of undue plasticity, swelling and caking properties cannot be coked by the ordinary briquetting and carbonization processes to produce a dense coked product. The improved results of the invention can be obtained in connection with any such coal by subjecting the hot pulverized coal at a temperature of between 115 and 150° C., dependent upon the coal and the final state of oxidation desired, and then subjecting it to an oxidizing gas at elevated pressures of from 20 to 150 lbs. pressure for 3 to 6 hours, again depending upon the coal and the final state of oxidation required. The coal so treated can be formed into briquettes and carbonized by any of the well known briquette carbonizing processes, at a temperature rise of at least  $2\frac{1}{2}$ ° C. per minute through the plastic temperature range and without interference from swelling and caking.

## What I claim is:

1. A method of coking badly swelling and caking coals which comprises pulverizing and drying the coal and then subjecting it to a controlled oxidation treatment in the presence of air pressure of from 45 to 150 lbs. per square inch and at a temperature of from 115° to 200° C. depending upon the coal and the degree of oxidation required and subsequently converting said treated coal into coke by carbonizing at a temperature rise of about 2½° C. per minute through the plastic temperature range.
2. A method of coking badly swelling and caking coals which comprises pulverizing and drying the coal and then subjecting it to a controlled oxidation treatment in the presence of air pressure of from 45 to 150 lbs. per square inch and at a temperature of from 115° to 200° C. from 3 to 6 hours depending upon the coal and the degree of oxidation required and subsequently converting said treated coal into coke by carbonizing at a temperature rise of about 2½° C. per minute through the plastic temperature range.
3. A method of coking badly swelling and caking coals which comprises pulverizing the coal, drying the coal, and then subjecting it to a controlled oxidation treatment in the presence of air pressure of from 45 to 150 lbs. per square inch and at a temperature of from 115° to 200° C. from 3 to 6 hours depending upon the coal and the degree of oxidation required and subsequently converting said treated coal into coke by carbonizing at a temperature rise of about 2½° C. per minute through the plastic temperature range.
4. A method of coking Pittsburgh seam coal which comprises pulverizing the coal, drying in the atmosphere at 150° C. and then subjecting the dry coal to a controlled oxidation treatment in the presence of air pressure of 50 lbs. per square inch and at a temperature of 115° C., said pressure and temperature being maintained for a period of about 4 hours and subsequently converting said treated coal into coke by carbonizing at a temperature rise of about 2½° C. per minute through the plastic temperature range.
5. A method of making carbonized briquettes from coking coals which comprises subjecting a pulverized, substantially dry, badly swelling and caking coal to a controlled oxidation treatment in the presence of an oxidizing gas pressure of from 45 to 150 pounds per square inch and at a temperature of from 115° to 200° C. to effect a reduction of the swelling and caking properties thereof, subsequently compressing into briquettes and subjecting said briquettes to carbonization at a temperature rise of about 2½° C. per minute through the plastic temperature range.
6. A method of making carbonized briquettes from caking coals which cannot normally be compressed into briquettes and carbonized at a temperature rise of more than ½° C. per minute through the plastic temperature range without badly swelling and caking, which comprises the steps of pulverizing and drying said coal and then subjecting the dried, pulverized coal to a controlled oxidation treatment in the presence of air pressure of from 45 to 150 pounds per square inch and at a temperature of from 115 to 200° C. to effect a reduction of the swelling and caking properties thereof, forming briquettes of said treated coal and subjecting the briquettes to a carbonization treatment at a temperature rise of at least 2½° C. per minute through the plastic temperature range.
7. A process according to claim 6 in which the pulverized coal is subjected to oxidation in the presence of air pressure of about 50 lbs. per square inch and at a temperature of about 150° C. for a period of about 4 hours.
8. A process according to claim 6 in which sulfite liquor is used as a binder in the formation of briquettes.
9. A process according to claim 6 in which molasses is used as a binder in the formation of briquettes.
10. A process according to claim 6 in which coal tar is used as a binder in the formation of briquettes.

WILLIAM JOSEPH KRUPPA.